

## UNITED STATES PATENT OFFICE

2,190,290

PROCESS FOR PREPARING ALLOYS OF  
CALCIUM WITH ALUMINUM

Gustaf Newton Kirsebom, Westbury-on-Trym,  
Bristol, England, assignor to Calloy Limited,  
London, England, a joint-stock company of  
England

No Drawing. Application February 9, 1938,  
Serial No. 189,592. In Great Britain February  
11, 1937

1 Claim. (Cl. 75—135)

In the specification of my prior United States Patent No. 1,935,245 a process is described for the preparation of aluminum alloys including alkaline earth metal alloys, a specific application of which process comprises heating an alkaline earth metal oxide or carbonate in a molten bath of aluminum below the surface thereof; for example, by placing on the top of a bath of molten aluminum, pieces of alkaline earth metal 5 oxide or carbonate of sufficient size to overcome the surface tension of molten aluminum and sink below the surface.

In describing the carrying out of the said process of my prior patent, a temperature range 15 was given as between 700 and 1500° C., and when working the process in order to obtain the residues in the form of unfused dross, a range of from 1000 to 1200° C. was given, and when working, within this last-named range of from 20 1000—1200° C., in the case of the preparation of calcium aluminum alloys from lime, the calcium oxide was reduced to metallic calcium which alloyed with the excess aluminum, and the aluminum oxide obtained as a result of this reduction 25 formed a dross which separated out round the sides and at the bottom of the crucible. Such dross entrained a certain amount of aluminum alloy, and it was necessary to treat the dross in a separate process for the recovery of aluminum 30 num therefrom.

Now, according to the present invention, alkaline earth metal oxides or carbonates or similar oxygen-containing compounds are heated in a bath of molten aluminum below the surface of 35 the latter at such a high temperature (as hereinafter indicated) that, while an alloy of aluminum and alkaline earth metal is formed, the residue of the mass is fused and converted into the form of a molten slag which latter constitutes a separate layer beneath the molten alloy of aluminum and alkaline earth metal.

The temperature to which the aluminum and alkaline earth metal compound must be heated 40 in order to obtain the formation of a molten slag depends upon the alkaline earth metal compound used. Thus, calcium aluminate,



formed when a calcium compound is used has a 45 melting point about 1350° C.; and in the case of strontium and barium compounds the aluminates thereof melt at about 1400° C.; while magnesium aluminate does not melt until 1800° C. However, a working temperature between 1350 50 and 1600° C., may be employed, for example,

1550° C.; and if the slag material present is one which would not be freely molten within this temperature range, calcium aluminate can be added thereto as a fluxing agent or there may be used as starting material, an alkaline earth metal compound containing lime, (for example dolomite) but in this case, calcium will also be introduced into the magnesium or other alkaline earth metal.

The present invention will now be described 10 with reference to the preparation of specific alkaline earth-aluminum alloys.

In the case of calcium-aluminum alloys, lime 15 may conveniently be introduced on to the top of the bath of molten aluminum, heated (in any suitable furnace) to a temperature near to, but below the boiling point of aluminum, advantageously a temperature of 1500—1600° C.; the lime being in the form of pieces of sufficient size 20 to overcome the surface tension of molten aluminum (for example, pieces ranging in size from 1 mm. to 100 mm.). Under these circumstances, the following reaction takes place:



The process can be carried out continuously as the aluminum alloy floats at the top of the calcium aluminate slag, and if the metal and slag be tapped at different levels from time to time, there is no need to interrupt the process.

This invention may advantageously be carried 30 into practice by employing an electric arc furnace or an electric high frequency induction furnace and may be worked as a continuous process as aforesaid; or if desired may be worked 35 as a "batch" process in any suitable electric or other furnace.

The following is an example of the procedure which may be adopted in preparing a calcium-aluminum alloy in accordance with the invention 40 when working as a "batch" process:

70 lbs. of aluminum and 50 lbs. of lime, the latter in pieces e. g. ranging from a few mm. diameter to walnut size, are heated together in an electric arc furnace to a temperature of 45 1500—1600° C., for example, 1550°, i. e. near to, but below, the boiling point of aluminum. The pieces of lime sink into the molten aluminum and reduction takes place with the formation of metallic calcium which alloys with the excess 50 aluminum. There is thus obtained 75 to 76 lbs. of a calcium-aluminum alloy containing 20—25% of calcium and about 45 lbs. of calcium aluminate slag. In thus working as a "batch" process, at the before-mentioned temperatures, the re- 55

duction will be completed in about three quarters of an hour.

The process may be carried out continuously by tapping off some of the aluminum alloy from the upper part of the furnace and some of the calcium aluminate slag from or near the bottom of the furnace, and a further charge added without interruption of the process.

Apart from the advantage of obtaining a clean separation of the metal alloy from the slag, the slag produced in this case is a marketable product and can (in an inexpensive manner, e. g. by grinding) be used for the preparation of cements

such as "ciment fondu", and thus avoid any expensive treatment of the slag for the recovery of aluminum.

What I claim is:

A process for preparing alloys of calcium with aluminum, which comprises heating lime in a bath of molten aluminum below the surface of the latter wherein the temperature of the bath is maintained between 1500 and 1600° C. and calcium aluminate is allowed to collect below 10 the molten bath of calcium-aluminum alloy formed.

GUSTAF NEWTON KIRSEBOM.